

3,136,629

**PRODUCTION OF URANIUM-CARBON ALLOYS**  
 Jack Williams, Abingdon, and Michael Colin Regan, Botley, England, assignors to United Kingdom Atomic Energy Authority, London, England  
 No Drawing. Filed Sept. 2, 1960, Ser. No. 53,635  
 Claims priority, application Great Britain Sept. 8, 1959  
 9 Claims. (Cl. 75—122.7)

The invention relates to the production of dense uranium-carbon alloys.

It is known from United States Patent No. 2,569,225 and British Patents Nos. 825,041 and 821,287 to produce uranium-carbon alloys containing varying proportions of uranium carbides and of differing structures, from mixtures of uranium and carbon. A preferred method of producing such alloys is to heat a cold-compacted mixture of uranium and carbon powders to a temperature of 800° to 1125° C. to cause a solid-state reaction between the uranium and carbon. Alloys produced by this method, however, have a density only about 90-93% of theoretical and an "open" porosity of 1 to 1½%.

According to the present invention a method of producing a dense uranium-carbon alloy, which may also comprise plutonium, comprises cold-compacting and then sintering at a temperature of at least 800° C., a mixture of uranium powder and carbon powder (and if desired plutonium powder) containing also iron in the form of an intermetallic compound of iron and uranium, the iron constituting from 1 to 10% of the whole by weight. The intermetallic compound may be  $UFe_2$  or  $U_6Fe$ , use of the latter being limited to iron contents less than 3.8% of the whole by weight. The preferred intermetallic compound is  $UFe_2$  since we have found that it gives the highest alloy density. The amounts of  $UFe_2$  corresponding to 1% and 10% by weight of iron are 3.1% and 31% respectively. The amount of  $U_6Fe$  corresponding to 1% by weight of iron is 26.5%. We have found that maximum density is attained when the iron content of the mixture is about 3% by weight of the whole. This is achieved, for example, when the amount of  $UFe_2$  used is about 10% by weight of the whole.

The uranium-carbon alloys which can be produced according to this invention may also include plutonium which may replace part of the uranium powder in the starting mixture.

We have found further, that when  $UFe_2$  is used as the intermetallic compound, the maximum density as a percentage of the theoretical density, and also the minimum "open" porosity, is attained when the carbon content of the mixture is in the stoichiometric proportion to the uncombined uranium content to form uranium monocarbide, i.e., 4.8% by weight of the total of uncombined uranium and carbon.

Heating of the cold compacted mixture to effect the sintering thereof must be performed at a temperature in excess of 800° C., which is the known temperature at which a solid state reaction takes place between uranium and carbon. However, the heating of the cold compacted mixture is preferably achieved very rapidly in accordance with the teachings set forth in our copending U.S. patent application Serial No. 53,634, filed September 2, 1960. As set forth in the aforesaid application, the cold compacted mixture of uranium powder, carbon powder, and intermetallic compound of iron and uranium is heated to a sintering temperature by plunging the mixture into a furnace heated to a temperature of 1000° C. to 1125° C. whereby the heat of reaction of the mixture sintering furnace causes its temperature to rise above the melting point of uranium. We have found that the rate of rise of temperature of the compacted mixture when it is plunged into the furnace is very rapid and depends upon

the size of the compact. It is certainly greater than 100° C. per minute, and may be as high as 500° C. per minute for small compacts. The actual temperature reached by the compact depends upon the size of the compact, but is within the range 1200 to 1450° C.

5 The nature of the invention will be made more apparent by the following examples.

#### EXAMPLES I TO VI

Uranium powder of particle size to pass a 300 mesh 10 British standard test sieve was mixed with ultrafine graphite in proportions of 95.2% uranium powder to 4.8% graphite, by weight. Samples of this mixture were mixed with amounts of  $UFe_2$  varying from 5 to 30% by weight of the whole. The mixtures of uranium, graphite and  $UFe_2$  were then cold-compacted at 60 tons/sq. in. in a tungsten carbide-lined die to form compacts of various sizes. Each compact was placed in an alumina boat and passed rapidly into a vacuum furnace heated to 1100° C. Each compact was estimated to reach a maximum temperature of 1200° to 1450° C. within a few minutes due to the heat of reaction, and was then heated at 1100° C. for 2 hours. The densities and porosities of the products are given in the following table, in which a product containing no  $UFe_2$  but produced by the same method is included for comparison.

Table I

| Example | Weight percent of whole |      |      | Density (gm./cc.) |          | Porosity (percent) |      |
|---------|-------------------------|------|------|-------------------|----------|--------------------|------|
|         | $UFe_2$                 | C    | Fe   | Theoretical       | Measured | Total              | Open |
| I       | 0                       | 4.80 | 0    | 13.63             | 12.40    | 9.0                | 0.81 |
| II      | 5                       | 4.58 | 1.57 | 13.61             | 12.85    | 5.5                | 0.84 |
| III     | 10                      | 4.32 | 3.13 | 13.59             | 13.09    | 3.7                | 0.36 |
| IV      | 15                      | 4.08 | 4.70 | 13.57             | 13.04    | 4.5                | 0.48 |
| V       | 20                      | 3.84 | 6.27 | 13.55             | 12.95    | 4.5                | 0.30 |
| VI      | 25                      | 3.60 | 7.83 | 13.53             | 12.85    | 5.0                | 0.30 |
|         | 30                      | 3.36 | 9.40 | 13.51             | 12.76    | 5.7                | 0.59 |

40 Table I shows that for  $UFe_2$  contents between 5 and 30% (iron contents 1.57 to 9.40%) the density is substantially higher than the density when no  $UFe_2$  is used, and that the highest density and lowest total porosity is achieved when the  $UFe_2$  content is 10%. Furthermore the open porosity is substantially reduced when the  $UFe_2$  content is 10% or more.

#### EXAMPLES VII TO XII

50 Similar mixtures to those of Examples I to VI were cold-compacted and sintered as before, except that the proportions of uranium powder and graphite were 95.0% and 5.0% respectively. The results obtained are shown in the following table:

| Example | Weight percent of whole |      |      | Density (gm./cc.) |          | Porosity (percent) |      |
|---------|-------------------------|------|------|-------------------|----------|--------------------|------|
|         | $UFe_2$                 | C    | Fe   | Theoretical       | Measured | Total              | Open |
| VII     | 0                       | 5.0  | 0    | 13.50             | 12.34    | 9.5                | 1.19 |
| VIII    | 5                       | 4.75 | 1.57 | 13.49             | 12.74    | 5.6                | 1.07 |
| IX      | 10                      | 4.50 | 3.13 | 13.48             | 12.87    | 4.4                | 0.77 |
| X       | 15                      | 4.25 | 4.70 | 13.46             | 12.84    | 4.4                | 0.65 |
| XI      | 20                      | 4.00 | 6.27 | 13.44             | 12.76    | 5.1                | 0.74 |
| XII     | 25                      | 3.75 | 7.83 | 13.42             | 12.75    | 5.0                | 0.59 |
|         | 30                      | 3.50 | 9.40 | 13.41             | 12.60    | 6.1                | 0.65 |

Table II shows similar results to those of Table I.

#### EXAMPLES XIII-XVIII

Similar mixtures to those of Examples II and VIII were

cold-pressed and sintered as before, except that the proportion of uranium powder was varied from 96.0 to 94.6% and that of graphite correspondingly from 4.0 to 5.4%. The results obtained are shown in the following table:

Table III

| Example | Weight percent carbon— |          | Density (gm./cc.) |          | Porosity (percent) |      |
|---------|------------------------|----------|-------------------|----------|--------------------|------|
|         | of U/C mixture         | of whole | Theoretical       | Measured | Total              | Open |
| XIII    | 4.0                    | 3.60     | 14.15             | 13.26    | 6.3                | 0.80 |
| XIV     | 4.2                    | 3.18     | 14.00             | 13.25    | 5.4                | 0.62 |
| XV      | 4.4                    | 3.96     | 13.86             | 13.18    | 4.9                | 0.43 |
| XVI     | 4.6                    | 4.14     | 13.73             | 13.12    | 4.4                | 0.55 |
| II      | 4.8                    | 4.32     | 13.59             | 13.09    | 3.7                | 0.36 |
| VIII    | 5.0                    | 4.50     | 13.43             | 12.87    | 4.4                | 0.77 |
| XVII    | 5.2                    | 4.68     | 13.28             | 12.62    | 5.0                | 1.35 |
| XVIII   | 5.4                    | 4.86     | 13.16             | 12.38    | 5.9                | 1.64 |

Table III shows that the maximum density as a percentage of the theoretical density (as shown by the minimum total porosity) is achieved when the carbon content is 4.8% of the U/C mixture, i.e. the stoichiometric proportion to form uranium monocarbide.

The sintered products of Examples I to VI consist of uranium mono-carbide (UC) in intimate mixture with  $UFe_2$  in the interstices between the UC particles. In those containing excess uranium i.e. the products of Examples XIII to XVI, the interstices contain a composition intermediate between U and  $UFe_2$ . In those containing excess carbon i.e. the products of Examples VII to XII, XVII and XVIII, the interstices contain a composition which consists of carbon and  $UFe_2$ , which may react to form further UC and free iron.

## EXAMPLE XIX

A mixture of 74.2% uranium powder and 25.8% graphite was mixed with  $U_6Fe$  powder in an amount such that the  $U_6Fe$  constituted 83.3% of the whole by weight. In this composition the iron content of the mixture was 3.13% and the carbon content 4.32%, as in Example II. The composition was cold-compressed and sintered as before. The product had a density of only 12.20 gm./cc., but was of similar constitution to that of Example II, i.e. uranium monocarbide in intimate mixture with  $UFe_2$  in the interstices between the UC particles.

We claim:

1. A method of producing a uranium-carbon alloy of high density and low porosity comprising mixing uranium powder, carbon powder, and iron in the form of an intermetallic compound of iron and uranium, the iron constituting from about 1 to 10% of the whole by weight,

4  
cold compacting the mixture, passing the mixture to a sintering zone, heating such zone to a temperature of between about 800° C. and 1125° C., and maintaining the mixture in such zone for a period of time sufficient to effect the complete sintering thereof.

2. A method for producing a uranium-carbon alloy of high density and low porosity comprising mixing uranium powder, carbon powder, and iron in the form of an intermetallic compound of iron and uranium, the iron constituting from about 1 to 10% of the whole by weight, cold compacting the mixture, passing the compacted mixture to a sintering zone maintained at the time of passing of the mixture at a temperature within the range of about 1000–1125° C., permitting the temperature in the sintering zone to rapidly rise for a short period of time solely as a result of the exothermic heat generated by the reaction of the mixture at a rate greater than about 100° C. per minute to a temperature between about 1200–1450° C., and thereafter heating the mixture in said sintering zone at a temperature of about 1000–1125° C. for a period of time sufficient to effect a complete sintering of the mixture.

3. A method according to claim 2, in which the iron constitutes about 3% of the whole by weight.

4. A method according to claim 2, in which the iron constitutes less than 3.8% of the whole by weight and the said intermetallic compound is  $U_6Fe$  comprising at least 26.5% of the whole by weight.

5. A method according to claim 2, in which the said intermetallic compound is  $UFe_2$  comprising 31.1% to 31% of the whole by weight.

6. A method according to claim 5, in which the  $UFe_2$  comprises about 10% of the whole by weight.

7. A method according to claim 2 in which the uranium powder and carbon powder in the said mixture are in the stoichiometric proportion to form uranium monocarbide.

8. A method in accordance with claim 2, wherein plutonium metal powder is mixed with the uranium powder, carbon powder, and iron.

9. A formed uranium-carbon alloy of high density and low porosity consisting essentially of an intimate sintered mixture of uranium monocarbide particles with the compound  $UFe_2$  in the interstices between the particles, the portion of iron in said alloy being between about 1 to 10% by weight.

## References Cited in the file of this patent

## UNITED STATES PATENTS

|    |           |        |                |
|----|-----------|--------|----------------|
| 50 | 2,526,805 | Carter | Oct. 24, 1950  |
|    | 2,569,225 | Carter | Sept. 5, 1951  |
|    | 2,807,542 | Frank  | Sept. 24, 1957 |